# EUROPEAN PATENT SPECIFICATION

(11) **EP 2 808 094 B1**
(45) Date of publication and mention of the grant of the patent: **18.09.2019**
(21) Application number: 14169142.8
(22) Date of filing: 20.05.2014
(51) Int. Cl.: B05D 1/32, B05D 5/06, B05D 1/02, B05D 5/00

(54) **Colored aluminum article producing method**
Herstellungsverfahren für gefärbten Aluminiumartikel
Procédé de production d'article en aluminium coloré

(30) Priority: 27.05.2013 JP 2013110572
(43) Date of publication of application: 03.12.2014
(73) Proprietor: Mimaki Engineering Co., Ltd., Tomi-shi, Nagano 389-0512 (JP)
(72) Inventor: Nakamura, Norikazu, Tomi-shi, Nagano 389-0512 (JP); Tabayashi, Isao, Tomi-shi, Nagano 389-0512 (JP); Ohnishi, Masaru, Tomi-shi, Nagano 389-0512 (JP)
(74) Representative: Fédit-Loriot

(56) References cited:
- GB-A- 2 478 641
- US-A1- 2012 171 807

## Description

### Technical Field

The present invention relates to a colored aluminum article producing method, a coloring method, and a liquid ejection apparatus.

### Background Art

Aluminum materials such as aluminum subjected to an anodizing process (alumite process) have been widely used. For example, a method is known that colors such aluminum materials. In this method, an aluminum material with an anodized coating is subjected to an etching process in a dilute alkaline aqueous solution to chemically dissolve the surface of the exposed portion of a barrier layer at the bottom portion in the pores of the anodized coating. The aluminum material is then colored either electrolytically in a metal salt-containing electrolytic coloring bath, or by being dipped in a pigment dispersion to allow pigment particles to electrophoretically migrate and deposit inside the pores of the anodized coating (see, for example, PTL 1).

### Citation List

### Patent Literature

PTL 1: JP-A-11-236697

Besides, GB 2 478 641 A discloses an object comprising several surfaces, part of which is provided with mask means and part of which does not have mask means and has a coating, wherein the mask means comprises a PTFE and the coating includes a plating deposition coating.

Further US 2012/171 807 A1 discloses a method and an apparatus for masking of substrates for deposition, and subsequent lifting of the mask with deposited material.

### Technical Problem

In the method disclosed in PTL 1, colors are provided electrolytically, or by electrophoretic migration and deposition of pigment particles. However, there are increasing demands for more appropriate coloring methods (for example, a faster coloring method, and a low-cost coloring method), for example, in manufacture of industrial products. It is accordingly an object of the present invention to provide a colored aluminum article producing method, a coloring method, and a liquid ejection apparatus intended to solve the foregoing problem.

### Solution to Problem

After intensive studies, the inventors of the present application found an efficient way to appropriately color aluminum materials with a dye, using a mask formed with a liquid ejection head that ejects liquid using the inkjet system. The present invention includes the following configurations to solve the foregoing problem.

### (Configuration 1)

A method for producing a colored aluminum article by coloring an aluminum material, the method including: a mask forming step of forming a defined region coating mask that covers a pre-defined region of the aluminum material; a coloring step of coloring the aluminum material with a dye in a region not covered by the defined region coating mask; and a mask detaching step of detaching the defined region coating mask from the aluminum material after the coloring step, wherein, in the mask forming step, a mask forming liquid as a liquid for forming the defined region coating mask is ejected onto the aluminum material with a liquid ejection head that ejects liquid using an inkjet system.

With this configuration, by using the liquid ejection head to form the defined region coating mask, the defined region coating mask can be appropriately formed in a shorter time period and at lower cost compared to, for example, forming the defined region coating mask by using the photomask technique. Further, because a dye is used to color the aluminum material, colors can be provided more easily and more appropriately than in methods, for example, such as the electrolytic coloring, and the electrophoretic migration and deposition of pigment particles. The foregoing configuration can thus appropriately color, for example, aluminum materials, for example, in a short time period and at low cost.

As used herein, "aluminum material" is, for example, an aluminum member with an anodized coating formed in at least a region where a color is to be provided. The aluminum material may be aluminum subjected to an anodizing process (alumite process). The aluminum in this process is preferably subjected to, for example, an oxidation treatment with an acidic liquid such as sulfuric acid.

### (Configuration 2)

In the mask forming step, an acrylic UV curable ink is used as the mask forming liquid, and the liquid ejection head ejects the mask forming liquid to the pre-defined region to form the defined region coating mask. In the coloring step, a dye solution that uses a solvent capable of dissolving the dye, or that uses water as a solvent is used to color the region not covered by the defined region coating mask. In the mask forming step, the defined region coating mask is formed, for example, by curing the mask forming liquid with ultraviolet light that is irradiated after the liquid has landed on the aluminum material.

When a dye solution (dye ink) is used to color the region not covered by the defined region coating mask, the defined region coating mask must satisfy the condition that the dye does not permeate underneath the defined region coating mask. The defined region coating mask is also required to be insoluble in the dye solvent (solvent), and easily detachable after the coloring. The present inventors found that the defined region coating mask which appropriately satisfies these conditions can be formed when an acrylic UV curable ink is used as the mask forming liquid in using a dye that uses a solvent capable of dissolving the dye (organic solvent), or that uses water as a solvent (hereinafter, collectively referred to as "dye dissolvable solvent").

More specifically, for example, pigment particles used to provide colors typically have larger molecular sizes than the molecules forming the dye color. Thus, when a pigment color is used, only the unmasked region can be appropriately colored after masking the region where a color is not required.

The present inventors found that the dye used to provide a color tends to seep between the mask and the aluminum material, and undesirably color a part of the masked region because the dye molecules dissolved in the solvent are smaller than the size of pigment particles. It was also found that such a dye seeping phenomenon occurs, for example, when the mask durability, which varies with the mask material, becomes weaker on the aluminum material, or when the adhesion between the mask and the aluminum material is insufficient.

After intensive studies, the present inventors found that the durability of the defined region coating mask on the aluminum material can be sufficiently improved, and sufficient adhesion can be provided between the aluminum material and the defined region coating mask to appropriately prevent dye permeation when an acrylic UV curable ink is used as the mask forming liquid with a dye that uses a dye dissolvable solvent, as noted above. It was also found that the defined region coating mask with the foregoing configuration does not dissolve in the dye solvent (solvent), and can easily be detached after the coloring. The foregoing configuration can thus more appropriately form the defined region coating mask, for example, when the dye uses a dye dissolvable solvent. This makes it possible to more appropriately color the aluminum material.

The requirement for the defined region coating mask not to permeate the dye is, for example, the requirement for the dye not permeate to the region covered with the defined region coating mask to such an extent as may be decided by the required color accuracy. Being insoluble in the dye solvent (solvent) does not necessarily mean that the defined region coating mask is completely insoluble, and, for example, the term is inclusive of the defined region coating mask being partially dissolved to such an extent that the defined region coating mask can exhibit its function in the coloring step. Being "easily detachable after the coloring" means that, for example, the defined region coating mask can be appropriately detached in the mask detaching step with, for example, a remover such as IPA (isopropyl alcohol) . Preferred for use as the acrylic UV curable ink is, for example, an ink that contains 50 weight% or more of an acrylic acid ester.

### (Configuration 3)

In the mask forming step, a UV curable ink of the property to stretch after curing is used as the mask forming liquid, and the liquid ejection head ejects the mask forming liquid to the pre-defined region to form the defined region coating mask. The UV curable ink of the property to stretch after the curing is, for example, a UV curable ink that turns itself into an elastic resin after being cured.

With this configuration, for example, the adhesion between the defined region coating mask and the aluminum material can be more appropriately improved. It is also possible to more appropriately satisfy the requirement for the defined region coating mask not to permeate the dye underneath the mask. With the foregoing configuration, the defined region coating mask also can become more easily detachable after the coloring. The foregoing configuration can thus more appropriately form the defined region coating mask.

### (Configuration 4)

In the mask forming step, an acrylic UV curable ink is used to form the defined region coating mask on the aluminum material etched with an acidic solution. The etching is, for example, the process that dissolves the surface of the exposed portion of a barrier layer at the bottom portion in the pores of the anodized coating of the aluminum material. Preferred for use as the acidic solution is, for example, a sulfuric acid solution.

After intensive studies, the present inventors found that the alkali resistance can become smaller depending on the type of the ink composition of the acrylic UV curable ink used as the material of the defined region coating mask. It was also found that the dye has the risk of passing through the defined region coating mask when the coloring step is performed in a certain manner. For example, when the acrylic UV curable ink used has the property to greatly stretch after the curing (for example, 200% or greater stretch), the very high softness of the ink may make the cured coating of the defined region coating mask poorly alkali resistant when a color is provided under alkaline pH in the coloring step, with the result that the dye passes through the defined region coating mask.

With the foregoing configuration, however, the coloring pH in the coloring step can be appropriately brought to a neutral pH range (for example, about pH 6 to 8), for example, as compared to using an aluminum material that is etched with an alkaline aqueous solution. The foregoing configuration can thus appropriately prevent the passage of the dye through the defined region coating mask even when, for example, the defined region coating mask has small alkali resistance. This makes it possible to more appropriately color the aluminum material.

### (Configuration 5)

The mask forming step includes forming a first mask with the mask forming liquid ejected to a region other than the pre-defined region in the target coloring region of the aluminum material where a color is to be provided, the first mask being formed to cover the region other than the pre-defined region; and applying a material liquid of the defined region coating mask to the aluminum material having the first mask, and removing the first mask to form the defined region coating mask in the pre-defined region.

With this configuration, the defined region coating mask is formed by using the first mask formed under the inkjet system, instead of being directly formed using the inkjet system. Accordingly, with the foregoing configuration, the defined region coating mask also can be formed by using a method other than the inkjet system. For example, the defined region coating mask may be formed by spray coating a material liquid of the defined region coating mask after forming the first mask. With this configuration, various types of liquids may be used as a material of the defined region coating mask, in addition to liquids that are ejectable using the inkjet system. It becomes also possible to freely choose a defined region coating mask material from different materials, for example, materials having strong resistance to the dye solution. The foregoing configuration can thus more appropriately form the defined region coating mask, for example. This makes it possible to more appropriately color the aluminum material.

With the foregoing configuration, the mask forming liquid is not directly used to form the defined region coating mask, but is used to form the first mask and thereby indirectly form the defined region coating mask. Preferably, the first mask is formed of, for example, a material that does not dissolve in the material of the defined region coating mask. Preferably, the material of the mask forming liquid is, for example, a liquid that fixes to the aluminum material in an undissolved form in the material liquid of the defined region coating mask.

### (Configuration 6)

The mask forming step includes: a rim forming step of forming a rim of the defined region coating mask with a first mask forming liquid for which a UV curable ink is used; and an inner region forming step of forming a mask inner region surrounded by the rim of the defined region coating mask, using a second mask forming liquid for which an ink is used that requires evaporation of solvent for fixing itself to the aluminum material. In the rim forming step, a first liquid ejection head for ejecting the first mask forming liquid is used to eject the first mask forming liquid to a region that becomes the rim of the defined region coating mask, and the first mask forming liquid landed on the aluminum material is irradiated with ultraviolet light to form the rim of the defined region coating mask. In the inner region forming step, a second liquid ejection head for ejecting the second mask forming liquid is used to eject the second mask forming liquid to the region surrounded by the rim formed in the rim forming step, and form the mask inner region of the defined region coating mask.

With this configuration, only the rim (edge) of the defined region coating mask pattern is UV cured in the rim forming step. Here, it is preferable to UV irradiate and cure the first mask forming liquid soon after the first mask forming liquid has landed on the aluminum material. With this configuration, for example, the rim of the defined region coating mask can be formed at high resolution. This makes it possible to appropriately form the defined region coating mask at high accuracy in the desired pattern.

According to the foregoing configuration, the inner pattern is formed in the inner region forming step, after the rim forming step. This makes it possible to sufficiently spread the dots of the second mask forming liquid landed on the aluminum material, as opposed to, for example, immediately curing the UV curable ink for formation of the inner pattern. The resulting inner pattern can thus have a pore-free homogeneous state. The foregoing configuration can thus more appropriately form the defined region coating mask, for example, in a homogenous fashion with high resolution.

Concerning the second mask forming liquid, the ink that requires evaporation of solvent for fixing itself to the aluminum material is, for example, an ink that requires removal of the solvent by heat drying or natural drying for fixing itself to the aluminum material. For example, a solvent UV ink, or a latex ink may preferably be used as the second mask forming liquid. It is also considered possible to use, for example, an ink containing resin capsules, or a solid ink that is solid at ordinary temperature.

### (Configuration 7)

A method for coloring an aluminum material, the method including: a mask forming step of forming a defined region coating mask that covers a pre-defined region of the aluminum material; a coloring step of dyeing the aluminum material in a region not covered by the defined region coating mask; and a mask detaching step of detaching the defined region coating mask from the aluminum material after the coloring step, wherein, in the mask forming step, a mask forming liquid as a liquid for forming the defined region coating mask is ejected onto the aluminum material with a liquid ejection head that ejects liquid using an inkjet system. The same effects obtained in, for example, configuration 1 also can be obtained with this configuration.

### (Configuration 8)

A liquid ejection apparatus for forming a defined region coating mask that covers a pre-defined region of an aluminum material, the apparatus including a liquid ejection head with which a mask forming liquid as a liquid for forming the defined region coating mask is ejected using an inkjet system, wherein the defined region coating mask covers the pre-defined region of the aluminum material in the coloring step that dyes the aluminum material, and is detached from the aluminum material after the coloring step. The same effects obtained in, for example, configuration 1 also can be obtained with this configuration.

### Advantageous Effects of Invention

The present invention can appropriately color an aluminum material, for example.

### Brief Description of Drawings

Fig. 1 is a flowchart representing an example of a colored aluminum article producing method according to an embodiment of the present invention.
Fig. 2 is a diagram explaining an example of a coloring mask, in which Fig. 2(a) is an exemplary configuration of a liquid ejection apparatus 10 used to form the coloring mask, Fig. 2(b) is an exemplary configuration of a coloring mask 102 formed on an aluminum material 20, and Fig. 2(c) is an exemplary configuration of the aluminum material 20 after being colored.
Fig. 3 is a diagram representing a first variation of coloring mask 102 formation, in which Fig. 3(a), (b), and (c) are examples of the steps of forming the coloring mask 102 in this variation.
Fig. 4 is a diagram representing a second variation of coloring mask 102 formation, in which Fig. 4(a) and (b) are examples of the steps of forming the coloring mask 102 in this variation.
Fig. 5 is a diagram representing exemplary methods of coloring the aluminum material 20 in full-color, in which Fig. 5(a) is a first example of coloring the aluminum material 20 in full-color, and Fig. 5(b) is a second example of coloring the aluminum material 20 in full-color.

### Description of Embodiments

Embodiments according to the present invention are described below with reference to the accompanying drawings. Fig. 1 is a flowchart of an example of a colored aluminum article producing method according to an embodiment of the present invention, representing exemplary steps of producing a colored aluminum article through dyeing of an aluminum material. The aluminum material is, for example, an aluminum member with an anodized coating formed in at least a region where a color is to be provided. The aluminum material may be aluminum (aluminum metal, or aluminum alloy) subjected to an anodizing process (alumite process). In this example, the colored aluminum article producing method includes at least a preparation step S102, a mask forming step S104, a coloring step S106, a mask detaching step S108, and a post-processing step S110. These steps may be the same or similar steps conventionally used for coloring aluminum materials, except for the following.

The preparation step S102 is a step of preparing an aluminum material to be colored. For example, an aluminum metal or aluminum alloy member is subjected to an anodizing process (alumite process) to prepare an aluminum material that has an anodized coating on the surface. Specifically, in the preparation step S102, a aluminum metal or aluminum alloy member is subjected to a series of processes that includes, for example, degreasing, water washing, etching, water washing, neutralization, electrolysis, and water washing to prepare an aluminum material for coloring. The etching is the process that dissolves the surface of the exposed portion of a barrier layer at the bottom portion in the pores of the anodized coating of the aluminum material, and is performed by, for example, an oxidation treatment that uses an acidic liquid such as sulfuric acid.

The mask forming step S104 is a step of forming a coloring mask that covers a region of the aluminum material where a color is not to be provided. In this example, the mask forming step S104 forms the coloring mask with the use of a liquid ejection apparatus that ejects a mask forming liquid as a liquid for forming the coloring mask. The liquid ejection apparatus is, for example, an apparatus that ejects liquid through a liquid ejection head using the inkjet head system. The coloring mask is an example of a defined region coating mask that covers a pre-defined region of the aluminum material. Formation of the coloring mask will be described later in greater detail.

The coloring step S106 is a step of dyeing the aluminum material in the region not covered by the coloring mask. In the coloring step S106, for example, the aluminum material with the coloring mask is dipped in a dye ink to color the aluminum material. The dye ink is a dye solution that uses a solvent capable of dissolving the dye, or that uses water as a solvent (dye dissolvable solvent). In this way, for example, the aluminum material can be appropriately colored in the region not covered by the coloring mask.

In the coloring step S106, for example, the aluminum material is placed in the dye ink filling a container. Various solvents, including organic solvents and water may be used as the dye dissolvable solvent, provided that colors can be appropriately provided. In the coloring step S106, it may be possible to dip the aluminum material in the dye ink, for example, by ejecting the dye ink to the aluminum material through a liquid ejection head. In this case, for example, the dye ink can be selectively ejected to locations requiring colors, and colors can be efficiently provided with less dye ink.

The mask detaching step S108 is a step of detaching the coloring mask from the aluminum material after the coloring step S106. In the mask detaching step S108, for example, the coloring mask is detached from the aluminum material with a remover such as IPA (isopropyl alcohol). The mask detaching step S108 may be performed, for example, by dipping the aluminum material in a remover for about 20 minutes.

The post-processing step S110 is a step of conditioning the surface of the colored aluminum material. The post-processing step S110 performs a series of processes that includes, for example, sealing, water washing, and drying to condition the aluminum material surface. The sealing is the process in which the fine pores of the alumite coating are sealed by heating with, for example, hot water and steam. After the sealing process, the dye can appropriately fix itself to the aluminum material. The subsequent washing and drying can appropriately clean the aluminum material surface.

According to the present example, for example, the liquid ejection head of the liquid ejection apparatus is used to form the coloring mask, and the coloring mask can be appropriately formed in a short time period and at low cost. Further, by using a dye, the aluminum material can be colored both easily and appropriately. The present example can thus appropriately color, for example, an aluminum material in a short time period and at low cost.

For convenience of explanation, descriptions have been given through the case where a single-color dye ink is used. It is also possible to use, for example, dye inks of more than one color when more than one color is to be provided. In this case, for example, the procedures of the mask forming step S104 to the mask detaching step S108 may be repeated a plurality of times to color the aluminum material with the dye ink of each color. In this way, more than one color can be appropriately provided. It is also considered possible to provide a partial decoration, for example, by performing the foregoing coloring procedures for an aluminum material that has a base color. It would also be possible to provide a full-color image by repeating the procedures of the mask forming step S104 to the mask detaching step S108 four times with dye inks of YMCK.

The mask forming step S104 to the mask detaching step S108 are described below in greater detail. Fig. 2 is a diagram explaining an example of the coloring mask, in which Fig. 2 (a) represents the configuration of a liquid ejection apparatus 10 used to form the coloring mask. In this example, the liquid ejection apparatus 10 includes a plurality of liquid ejection heads 12, ultraviolet sources 14, and a table 16.

The liquid ejection apparatus 10, for example, may have the same or similar configuration used by an inkjet printer. For example, a known inkjet printer may be used as the liquid ejection apparatus 10. Further, for example, the liquid ejection apparatus 10 may include components having the same configurations as those of a known inkjet printer.

The liquid ejection heads 12 represent a head unit that ejects liquid using the inkjet system. As an example, known inkjet heads may preferably be used as the liquid ejection heads 12. In the mask forming step S104 (see Fig. 1), the mask forming liquid as a liquid for forming the coloring mask is ejected onto an aluminum material 20 through at least one of the liquid ejection heads 12. This forms the coloring mask on the aluminum material 20.

As an example of its operation, the liquid ejection heads 12 perform a main scan operation in which the head 12 ejects the liquid as it moves in the predetermined Y direction, and a sub scan operation in which the head 12 moves relative to the aluminum material 20 in X direction orthogonal to Y direction as does, for example, the inkjet head of a known inkjet printer. In this way, the liquid ejection heads 12 eject the mask forming liquid for each different location of the aluminum material 20. In the mask forming step S104, for example, the mask forming liquid may be ejected by using two or more liquid ejection heads 12.

The ultraviolet sources 14 are light sources that produce ultraviolet light for curing a UV curable ink. In this example, the ultraviolet sources 14 are provided at the both ends of the liquid ejection heads 12 relative to Y direction, and cure the mask forming liquid landed on the aluminum material 20 through irradiation of ultraviolet light. The table 16 is a board-like member for mounting the aluminum material 20. The aluminum material 20 is mounted on the top surface on the table 16, opposite the liquid ejection heads 12.

According to the present example, the mask forming liquid can be appropriately ejected to the desired locations of the aluminum material 20, and the mask forming liquid landed on the aluminum material 20 can be appropriately cured. This makes it possible to appropriately form the coloring mask of the desired shape on the aluminum material 20.

Fig. 2(b) represents an exemplary configuration of a coloring mask 102 formed on the aluminum material 20. In this example, the aluminum material 20 is configured to include an aluminum metal portion 22 existing as aluminum metal, and an alumite coating 24 formed on the surface of the aluminum metal portion 22. In the mask forming step S104, the coloring mask 102 is formed so as to cover regions in portions of the alumite coating 24. Accordingly, the aluminum material 20 contacts the dye ink only in surface portions not covered by the coloring mask 102 upon being dipped in the dye ink in the coloring step S106. The dye ink thus colors only the regions not covered by the coloring mask 102.

Fig. 2(c) is a diagram of an exemplary configuration of the aluminum material 20 after being colored, representing an exemplary state of the aluminum material 20 after the post-processing step S110 (see Fig. 1). As shown in the figure, the aluminum material 20 is dyed only in portions other than the regions covered by the coloring mask 102. The present example can thus appropriately color the desired regions of the aluminum material 20 according to the shape of the coloring mask 102 formed.

The mask forming liquid and the dyeing solution (dye ink) used in the present example are described below in greater detail. When the region not covered by the coloring mask 102 is to be colored with the dye solution as in this example, the coloring mask 102 is required not to permeate the dye underneath the coloring mask 102 (non-permeable to the colorant), not to dissolve in the dye solvent (solvent), and to be easily detachable after the coloring. The coloring dye is used in the form of a solution of dye molecules smaller than the size of pigment particles in the solvent. The dye thus has the risk of seeping into the region between the coloring mask 102 and the aluminum material 20, and undesirably color a part of the region covered with the coloring mask 102, for example, when the durability of the coloring mask 102 on the aluminum material 20 is insufficient, or when the adhesion between the coloring mask 102 and the aluminum material 20 is insufficient. It is believed that the durability and the adhesion of the coloring mask 102 depend on, for example, the material used for the coloring mask 102.

The dye used in the dye solution of this example may be a dye that is soluble in water, or a dye that is soluble in an organic solvent. Specific examples of the dye that is soluble in water include acidic dyes, reactive dyes, anionic dyes such as direct dyes, basic dyes, disperse dyes, mordant dyes, and vat dyes. The disperse dye is, for example, a dye that enters the pores and dyes the object of interest. The mordant dye is, for example, a dye that forms an insoluble metal complex salt through reaction with metal to dye an object of interest. The vat dye is, for example, a dye such as an indigo dye. Examples of the dye that is soluble in an organic solvent include spirit dyes, and oil-soluble dyes.

Particularly preferred for use in this example are dyes that have excellent lightfastness, specifically, for example, premetallized dyes. Particularly preferred as aqueous premetallized dyes are, for example, azo or phthalocyanine premetallized acidic dyes. Other possible examples of the dye that is soluble in an organic solvent include spirit dyes that are soluble in polar solvents such as alcohol and ketone, and oil-soluble premetallized dyes that are soluble in aromatic hydrocarbon, glycol ether solvent, and the like. The dye solution, particularly the aqueous dye solution preferably contains a water-soluble organic solvent or a surfactant to improve the wettability and the permeability of the dye solution for the porous oxidation coating layer formed on the aluminum material surface.

When these dye solutions are used, it is preferable to use, for example, an acrylic UV curable ink as the mask forming liquid. For example, an ink containing 50 weight% or more of an acrylic acid ester may be used as the acrylic UV curable ink. Here, "ink" means a liquid that can be ejected through, for example, the liquid ejection heads 12 using the inkjet system. The ink may be a transparent ink, for example, such as a clear ink, or may be a color ink such as a color printing ink.

A specific composition of the mask forming liquid (acrylic UV curable ink) is preferably selected according to the type of the dye solution used. For example, when an aqueous dye solution is used, it may not be possible to obtain sufficient masking effect when the acid number of the UV curable ink is 100 or more under alkaline pH. It is preferable in this case to use an acryl component that does not have an acidic group.

With such a mask forming liquid, the durability of the coloring mask 102 on the aluminum material 20, and the adhesion between the coloring mask 102 and the aluminum material 20 can be appropriately improved with, for example, the dye ink that uses a dye dissolvable solvent. It is also possible to appropriately satisfy the requirement for the coloring mask 102 not to permeate the dye underneath the mask. The requirements not to dissolve in the dye solvent (solvent), and to be easily detachable after the coloring also can be appropriately satisfied. The present example can thus appropriately form the coloring mask 102 satisfying the various conditions.

A UV curable ink of the property to stretch after curing is preferably used as the mask forming liquid. The UV curable ink of the property to stretch after the curing is, for example, a UV curable ink that turns itself into an elastic resin after being cured. With this configuration, for example, the adhesion between the coloring mask 102 and the aluminum material 20 can be more appropriately improved. It is also possible to more appropriately satisfy the requirement for the coloring mask 102 not to permeate the dye underneath the mask. Further, with the foregoing configuration, the coloring mask 102 can become more easily detachable after the coloring. The coloring mask 102 can thus be more appropriately formed with the foregoing configuration.

For example, when the UV curable ink of the property to stretch after the curing has an excessively high stretch rate, the excessive softness may increase solubility in certain types of dye solvent (solvent) . It is therefore preferable that the UV curable ink of the property to stretch after the curing be, for example, an ink with a stretch rate of about 120 to 160%, more preferably an ink with a stretch rate of about 130 to 150%. The ink stretch rate of 120 to 160% (or 130 to 150%) means that the ink stretches, for example, at most 120 to 160% in terms of an area after being cured.

Preferred for use as the stretchable ink is, for example, a UV curable ink that contains 20 to 30 weight% of a multifunctional monomer (for example, hexamethylene diacrylate), and 55 to 65 weight% of a monofunctional monomer (for example, acrylic acid ester). Specific examples of the stretchable ink include the LF-140 UV curable ink available from Mimaki Engineering Co., Ltd. The LF-140 UV curable ink has a stretch rate of about 140%, and contains 55 to 65 weight% of an acrylic acid ester, 20 to 30 weight% of hexamethylene diacrylate, 10 to 15 weight% of a polymerizable initiator, 0.1 to 5 weight% of a pigment such as quinacridone magenta, and 0.1 to 5 weight% of additives. With the LF-140 UV curable ink used as the mask forming liquid, the coloring mask 102 can be appropriately prevented from dissolving in the dye ink solvent, and a clear color image can be appropriately obtained with, for example, the dye ink that contains a dye dissolvable solvent. It is also possible to appropriately satisfy the requirements for the coloring mask 102 not to permeate the dye underneath the mask, and to be easily detachable when IPA is used as the remover.

The UV curable ink of the property to stretch after the curing may be an ink that has an even greater stretch rate, for example, such as the LF-200 UV curable ink available from Mimaki Engineering Co., Ltd. The LF-200 UV curable ink has a stretch rate of about 200%, and contains isobonyl acrylate, an amine modified acrylic acid oligomer, tetrahydrofurfuryl acrylate, an initiator (diphenyl-2,4,6-trimethylbenzoylphosphine oxide), 2-(2-ethoxyethoxy)ethyl acrylate, an acrylic acid ester, and additives (sensitizer, dispersant, and polymerization inhibitor) . The coloring mask 102 also can be clearly formed also with such a mask forming liquid.

However, use of such a highly stretchable ink is potentially associated with increased solubility in the dye solvent because of the excessive ink softness, as noted above. For example, when the LF-200 UV curable ink is used, the alkali resistance of the cured coating may become insufficient, making the dye more permeable through the cured coating. It is therefore preferable to use an acidic solution, such as sulfuric acid, for the etching performed in the preparation step S102 of preparing the aluminum material 20 (see Fig. 1). In this case, for example, the pH of the coloring with the dye ink can be appropriately brought to a neutral pH range (for example, pH 6 to 8). This makes it possible to appropriately prevent the dye from passing through the coloring mask 102 even when the coloring mask 102 has a small alkali resistance.

When using the LF-200 UV curable ink, it is preferable to further heat the coloring mask 102 after the coloring mask 102 is cured by irradiation of ultraviolet light. In this way, for example, the hardness of the cured coating can be further improved. It is also possible to further increase the durability of the coloring mask 102. The heating effect can be obtained, for example, by several minutes of heating with a dryer. In order to more appropriately increase the hardness of the cured coating, it is preferable to apply heat with, for example, an oven at 50 to 60°C for about 1 hour.

Under certain coloring conditions or purposes, an ink that undergoes essentially no stretch after the curing may be used as the mask forming liquid, instead of using the UV curable ink of the property to stretch after the curing. The ink that undergoes essentially no stretch after the curing is, for example, a common UV curable ink whose components are not adjusted to make the ink stretchable. Preferred for use as such an ink is, for example, a hard UV curable ink.

In this case, the dye has increased durability against the dye solvent or the like, for example, as compared to using the stretchable ink, and the durability of the coloring mask 102 can be appropriately and sufficiently increased, for example, even when the coloring mask 102 has a small thickness. The thinner thickness of the coloring mask 102 makes it possible to form, for example, finer patterns with high accuracy. In this way, for example, colors can be appropriately provided at higher resolutions.

The hard UV curable ink may be, for example, the LH-100 UV curable ink available from Mimaki Engineering Co., Ltd. The LH-100 UV curable ink contains 50 to 60% of an acrylic acid ester, 30 to 35 weight% of hexamethylene diacrylate, 10 to 15 weight% of an initiator (diphenyl-2,4,6-trimethylbenzoylphosphine oxide), and 0.1 to 5% of additives.

With the hard UV curable ink, the coloring mask 102 can be appropriately prevented from dissolving in the dye ink solvent, and the requirements for appropriately obtaining a clear color image, and the requirement for the coloring mask 102 not to permeate the dye underneath the mask can be appropriately satisfied. However, the detachability of the coloring mask 102 may suffer compared to using the stretchable ink. It is therefore preferable to dip the aluminum material 20 in a remover for a longer time period in the detaching step S106 when a hard UV curable ink is used as the mask forming liquid.

Other than the foregoing inks, for example, a UV curable primer ink may be used as the mask forming liquid. Specific examples of such an ink include the PR-100 UV curable ink available from Mimaki Engineering Co., Ltd. The PR-100 UV curable ink contains 80 to 90% of an acrylic acid ester, 10 to 15 weight% of an initiator, and 0.1 to 5% of additives.

It should be noted, however, that using the PR-100 UV curable ink may lower the durability of the coloring mask 102 against the dye solvent or the like as compared to, for example, using the LF-140 or LH-100 UV curable ink. In this case, for example, the coloring mask 102 may dissolve in the dye solvent, and prevent a color from being appropriately provided.

When using the PR-100 UV curable ink, it is preferable to further heat the coloring mask 102 after the coloring mask 102 is cured by irradiation of ultraviolet light, as with the case of using the LF-200 UV curable ink described above. In this way, for example, the hardness of the cured coating can be further improved. This makes it possible to further increase the durability of the coloring mask 102.

The mask forming liquid may be, for example, an ink (liquid) other than the UV curable ink. Possible examples of such inks include solvent UV (SUV) inks prepared by adding a volatile organic solvent to a UV curable ink, and latex inks containing polymer materials such as an aqueous polymer. It is also considered possible to use inks containing resin capsules, or solid inks that are solid at ordinary temperature. The coloring mask of the desired shape also can be appropriately formed on the aluminum material 20 in this case by ejecting the ink on the aluminum material 20 with the liquid ejection heads 12. Solid inks (waxes: natural waxes such as carnauba wax, and beeswax; and synthetic waxes such as paraffin wax) also may be used as the mask material.

Variations of the coloring mask 102 formation in the mask forming step S104 are described below. Fig. 3 represents a first variation of the coloring mask 102 formation, in which Fig. 3(a), (b), and (c) are examples of the steps of forming the coloring mask 102 in this variation.

The formation of the coloring mask 102 of this variation is the same or similar to that described with reference to Figs . 1 and 2, except for the following. The liquid ejection apparatus 10 used in this variation has the same or similar configuration to that shown in Fig. 2(a).

In this variation, the mask forming liquid is used to form an intermediate mask 104, which is then used to form the coloring mask 102, instead of directly forming the coloring mask 102 with the mask forming liquid ejected through the liquid ejection heads 12 (see Fig. 2). The intermediate mask 104 is an example of the first mask that covers a region other than the pre-defined region.

Specifically, in the present variation, the mask forming liquid is ejected to regions other than the regions where the coloring mask 102 is to be formed, as shown in Fig. 3(a), and the liquid forms the intermediate mask 104 covering these regions (mask forming step S104). The regions other than the regions where the coloring mask 102 is to be formed are, for example, target coloring regions of the aluminum material 20 where a color is to be provided.

After forming the intermediate mask 104, a material liquid of the coloring mask 102 is applied to the aluminum material 20 to form a coloring mask material layer 106, as shown in Fig. 3(b). The material liquid of the coloring mask 102 may be applied, for example, by using a method other than the inkjet system. For example, the material liquid of the coloring mask 102 may be applied by spray coating. It is also possible to apply the material liquid of the coloring mask 102 using the inkjet system, using a liquid ejection head 12 different from that used to form the intermediate mask 104.

Thereafter, as shown in Fig. 3(c), the intermediate mask 104 is removed, leaving the coloring mask 102 material, and forming the coloring mask 102 of the predetermined pattern only in the regions where it is needed. In this configuration, the coloring mask 102 may be formed by using a method other than the inkjet system. The material of the coloring mask 102 thus may be any of various liquids other than liquids that are ejectable using the inkjet system. The material of the coloring mask 102 can thus be freely selected from a wide range of materials, for example, such as materials with strong resistance to the dye solution.

The intermediate mask 104 formed by the mask forming liquid is used specifically in the process of forming the coloring mask 102. Accordingly, the intermediate mask 104 is not required to have durability or other resisting properties against the dye ink solvent. The foregoing configuration thus enables use of various liquids also for, for example, the mask forming liquid ejected through the liquid ejection heads 12, provided that the liquid used does not dissolve in the material liquid of the coloring mask 102, and can fix itself to the aluminum material 20. The foregoing configuration can thus appropriately form the coloring mask 102, for example, and appropriately color the aluminum material 20.

Fig. 4 represents a second variation of the coloring mask 102 formation, in which Fig. 4(a) and (b) are examples of forming the coloring mask 102 in this variation. The formation of the coloring mask 102 of this variation is the same or similar to that described with reference to Figs. 1 and 2, except for the following. The liquid ejection apparatus 10 used in this variation has the same or similar configuration to that shown in Fig. 2(a).

In this variation, a rim forming step and an inner region forming step are performed in the mask forming step. The formation of the coloring mask 102 is thus a two-step process that includes formation of the rim, and formation of the inner region. A rim-forming first mask forming liquid, and an inner region-forming second mask forming liquid are used as the mask forming liquid. The first and second mask forming liquids are ejected through the designated heads in the liquid ejection heads 12 of the liquid ejection apparatus 10.

Specifically, a UV curable ink is used as the first mask forming liquid in this variation. In the rim forming step of the mask forming step S104, a first liquid ejection head 12 is used to eject the first mask forming liquid to a region that becomes the rim of the coloring mask 102, and the first mask forming liquid landed on the aluminum material 20 is irradiated with ultraviolet light with the ultraviolet sources 14 (see Fig. 2). This forms a rim 108 of the coloring mask 102, as shown in Fig. 4(a). In this manner, in this variation, only the rim (edge) of the coloring mask 102 pattern is UV cured in the rim forming step.

In the inner region forming step following the rim forming step, a second liquid ejection head 12 is used to eject the second mask forming liquid to the region surrounded by the rim 108 to form an inner region 110 of the coloring mask 102. In the present variation, an ink that requires solvent evaporation for fixing itself to the aluminum material 20 is used as the second mask forming liquid. The ink that requires solvent evaporation for fixing itself to the aluminum material 20 is, for example, an ink that requires removal of the solvent by heat drying or natural drying for fixing itself to the aluminum material 20. For example, a solvent UV ink, or a latex ink may preferably be used as the second mask forming liquid. It is also considered possible to use, for example, an ink containing resin capsules, or a solid ink that is solid at ordinary temperature.

This configuration makes it possible, for example, to sufficiently spread the dots of the second mask forming liquid landed on the aluminum material 20 inside the pattern of the coloring mask 102. The resulting inner pattern can thus have a pore-free homogeneous state. The foregoing configuration can thus more appropriately form the coloring mask 102, for example, in a homogenous fashion with high resolution.

In the rim forming step, it is preferable to irradiate ultraviolet light and cure the first mask forming liquid soon after it has landed on the aluminum material 20. With this configuration, for example, the rim of the coloring mask 102 can be formed at high resolution. This makes it possible to appropriately form the coloring mask 102 of the desired pattern with high accuracy.

The two-step formation of the coloring mask 102 by the rim forming step and the inner region forming step may be performed for, for example, only a region of the coloring mask 102, instead of the whole region. For example, a pattern may be formed with only the first mask forming liquid for a narrow region of the coloring mask 102. For regions that do not require high rim shape accuracy, a pattern may be formed only with the second mask forming liquid. In either case, the coloring mask 102 can be appropriately formed at high resolution in a homogenous fashion by forming different portions of the coloring mask 102 using methods that are suited for different portions.

More than one color may be given to the aluminum material by applications of the methods described with reference to Figs. 1 to 4. The following describes an example of such methods of providing more than one color.

Fig. 5 is a diagram representing exemplary methods of coloring the aluminum material 20 in full-color, in which Fig. 5(a) is a first example of coloring the aluminum material 20 in full-color, and Fig. 5(b) is a second example of coloring the aluminum material 20 in full-color.

As described in conjunction with Fig. 1, a full-color image can be provided, for example, by repeating the procedures of the mask forming step S104 to the mask detaching step S108 four times with dye inks of YMCK. In this case, for example, the inks of YMCK may be ejected into pores 202 of the alumite coating of the aluminum material 20 with the liquid ejection heads 12 (see Fig. 2) of the liquid ejection apparatus 10 (see Fig. 2) of the configuration shown in Fig. 2.

As a specific example, in this case, more than one color may be charged into a single pore 202 to overlay more than one color in the pore 202, as shown in Fig. 5 (a). With this configuration, various different colors can be used to realize full-color, for example, by appropriately overlaying inks of different colors YMCK. It is also possible, for example, to place inks of different colors side by side relative to the in-plane direction on the surface of the aluminum material 20 by charging only a single color to each different pore 202, as shown in Fig. 5(b). Also in this case, full-color can be realized, for example, in the same manner as in the common printing method employed by inkjet printers. The ink ejected through the liquid ejection heads 12 in this configuration may be a pigment ink.

Aside from the foregoing full-color methods of providing more than one color for the aluminum material 20, a method may be used that provides more than one color using specific colors. For example, two colors may be provided by repeating the procedures of the mask forming step S104 to the mask detaching step S108 of Fig. 1 twice with dye inks of two specific colors , for example, red and black. It is preferable in this case to, for example, define different color regions for the different dye inks in different portions of the aluminum material 20 so that these color regions intended for the different colors do not overlap. With this configuration, for example, two different colors can be more appropriately provided. In certain color applications, for example, the color regions of different colors may be overlaid either partially or completely. In this case, for example, a mesh mask may be used as the coloring mask to provide intermediate colors.

It is also possible to provide multiple (N) colors with greater numbers of dye inks of different colors. As an exemplary configuration, dye inks of different colors (for example, X1, X2) may be used in addition to the dye inks of two different colors, such as red and black. It is also preferable in this case to, for example, define different color regions for the different dye inks in different portions of the aluminum material 20 so that these color regions intended for the different colors do not overlap. With this configuration, for example, N different colors can be more appropriately provided. In certain color applications, for example, the color regions of different colors may be overlaid either partially or completely. In this case, for example, a mesh mask may be used as the coloring mask to provide intermediate colors.

While the embodiments of the present invention have been discussed in the foregoing detailed explanation, the technical scope of the present invention is in no way limited by the description of the embodiments above, and the embodiments may be altered or improved in many ways, as would be obvious to a person of ordinary skill in the art. An embodiment based on such alterations and improvements is encompassed in the technical scope of the present invention, as defined by the appended claims.

### Industrial Applicability

The present invention is suitable for, for example, methods of producing colored aluminum articles.

### Reference Signs List

- 10: Liquid ejection apparatus
- 12: Liquid ejection heads
- 14: Ultraviolet source
- 16: Table
- 20: Aluminum material
- 22: Aluminum metal portion
- 24: Alumite coating
- 102: Coloring mask (defined region coating mask)
- 104: Intermediate mask (first mask)
- 106: Coloring mask material layer
- 108: Rim
- 10: Inner region
- 202: Pore

## Claims

1. A method for producing a colored aluminum article by coloring an aluminum material using at least one liquid ejection head, the method comprising the steps of:
preparing an aluminum material on which an anodized coating is formed in at least a region where a color is to be provided;
forming a coloring mask that covers a region of the aluminum material where a color is not to be provided by using a UV curable ink;
coloring the aluminum material in the region not covered by the coloring mask with a dye solution that uses a solvent capable of dissolving the dye, or that uses water as a solvent;
detaching the coloring mask from the aluminum material after the coloring step, and
conditioning the surface of the colored aluminum material.

2. The method for producing a colored aluminum article according to claim 1, wherein the anodized coating contains fine pores and the conditioning step comprises sealing the fines pores of the anodized coating.

3. The method for producing a colored aluminum article according to claim 1 or 2, wherein the anodized coating contains fines pores and the conditioning step comprises sealing the fines pores of the anodized coating by heating.

4. The method for producing a colored aluminum article according to any one of claims 1 to 3, wherein the mask forming step comprises forming a defined region coating mask that covers a pre-defined region of the aluminum material.

5. The method for producing a colored aluminum article according to claim 4, wherein, in the mask forming step, an acrylic UV curable ink is used as the mask forming liquid, and the liquid ejection head ejects the mask forming liquid to the pre-defined region to form the defined region coating mask, and
wherein, in the coloring step, a dye solution that uses a solvent capable of dissolving the dye, or that uses water as a solvent is used to color the region not covered by the defined region coating mask.

6. The method for producing a colored aluminum article according to claim 4 or 5, wherein, in the mask forming step, a UV curable ink of the property to stretch after curing is used as the mask forming liquid, and the liquid ejection head ejects the mask forming liquid to the pre-defined region to form the defined region coating mask.

7. The method for producing a colored aluminum article according to any one of claims 4 to 6, wherein, in the mask forming step, an acrylic UV curable ink is used to form the defined region coating mask on the aluminum material etched with an acidic solution.

8. The method for producing a colored aluminum article according to any one of claims 4 to 7, wherein the mask forming step includes:
forming a first mask with the mask forming liquid ejected to a region other than the pre-defined region in the target coloring region of the aluminum material where a color is to be provided, the first mask being formed to cover the region other than the pre-defined region; and
applying a material liquid of the defined region coating mask to the aluminum material having the first mask, and removing the first mask to form the defined region coating mask in the pre-defined region.

9. The method for producing a colored aluminum article according to any one of claims 4 to 8, wherein the mask forming step includes:
a rim forming step of forming a rim of the defined region coating mask with a first mask forming liquid for which a UV curable ink is used; and
an inner region forming step of forming a mask inner region surrounded by the rim of the defined region coating mask, using a second mask forming liquid for which an ink is used that requires evaporation of solvent for fixing itself to the aluminum material,
wherein, in the rim forming step, a first liquid ejection head for ejecting the first mask forming liquid is used to eject the first mask forming liquid to a region that becomes the rim of the defined region coating mask, and the first mask forming liquid landed on the aluminum material is irradiated with ultraviolet light to form the rim of the defined region coating mask, and
wherein, in the inner region forming step, a second liquid ejection head for ejecting the second mask forming liquid is used to eject the second mask forming liquid to the region surrounded by the rim formed in the rim forming step, and form the mask inner region of the defined region coating mask.

## Patentansprüche

1. Verfahren zur Herstellung eines gefärbten Aluminiumgegenstandes durch Färben eines Aluminiummaterials unter Verwendung mindestens eines Flüssigkeitsausstoßkopfs, wobei das Verfahren die Schritte umfasst:
Vorbereiten eines Aluminiummaterials, auf dem eine eloxierte Beschichtung in mindestens einem Bereich ausgebildet wird, in dem eine Farbe bereitgestellt werden soll;
Ausbilden einer Färbemaske, die einen Bereich des Aluminiummaterials bedeckt, in dem eine Farbe nicht bereitgestellt werden soll, unter Verwendung einer UV-härtbaren Tinte;
Färben des Aluminiummaterials in dem Bereich, der nicht durch die Färbemaske bedeckt ist, mit einer Farbstofflösung, die ein Lösungsmittel verwendet, das in der Lage ist, den Farbstoff aufzulösen, oder die Wasser als Lösungsmittel verwendet;
Lösen der Färbemaske vom Aluminiummaterial nach dem Färbeschritt und
Aufbereiten der Oberfläche des gefärbten Aluminiummaterials.

2. Verfahren zur Herstellung eines gefärbten Aluminiumgegenstandes nach Anspruch 1, wobei die eloxierte Beschichtung feine Poren enthält und der Aufbereitungsschritt das Versiegeln der feinen Poren der eloxierten Beschichtung umfasst.

3. Verfahren zur Herstellung eines gefärbten Aluminiumgegenstandes nach Anspruch 1 oder 2, wobei die eloxierte Beschichtung fein Poren enthält und der Aufbereitungsschritt das Versiegeln der feinen Poren der eloxierten Beschichtung durch Erhitzen umfasst.

4. Verfahren zur Herstellung eines gefärbten Aluminiumgegenstandes nach einem der Ansprüche 1 bis 3, wobei der Maskenausbildungsschritt das Ausbilden einer einen definierten Bereich beschichtenden Maske umfasst, die einen vordefinierten Bereich des Aluminiummaterials bedeckt.

5. Verfahren zur Herstellung eines gefärbten Aluminiumgegenstandes nach Anspruch 4, wobei im Maskenausbildungsschritt eine UV-härtbare Acryltinte als Maskenausbildungsflüssigkeit verwendet wird und der Flüssigkeitsausstoßkopf die Maskenausbildungsflüssigkeit auf den vordefinierten Bereich ausstößt, um die einen definierten Bereich beschichtende Maske auszubilden, und
wobei im Färbeschritt eine Farbstofflösung, die ein Lösungsmittel verwendet, das in der Lage ist, den Farbstoff aufzulösen, oder die Wasser als Lösungsmittel verwendet, verwendet wird, um den Bereich zu färben, der nicht durch die einen definierten Bereich beschichtende Maske bedeckt ist.

6. Verfahren zur Herstellung eines gefärbten Aluminiumgegenstandes nach Anspruch 4 oder 5, wobei im Maskenausbildungsschritt eine UV-härtbare Tinte mit der Eigenschaft zum Dehnen nach dem Härten als Maskenausbildungsflüssigkeit verwendet wird und der Flüssigkeitsausstoßkopf die Maskenausbildungsflüssigkeit auf den vordefinieren Bereich ausstößt, um die einen definierten Bereich beschichtende Maske auszubilden.

7. Verfahren zur Herstellung eines gefärbten Aluminiumgegenstandes nach einem der Ansprüche 4 bis 6, wobei im Maskenausbildungsschritt eine UV-härtbare Acryltinte verwendet wird, um die einen definierten Bereich beschichtende Maske auf dem Aluminiummaterial auszubilden, das mit einer sauren Lösung geätzt wird.

8. Verfahren zur Herstellung eines gefärbten Aluminiumgegenstandes nach einem der Ansprüche 4 bis 7, wobei der Maskenausbildungsschritt umfasst:
Ausbilden einer ersten Maske, wobei die Maskenausbildungsflüssigkeit auf einen anderen Bereich als den vordefinierten Bereich im Zielfärbebereich des Aluminiummaterials ausgestoßen wird, in dem eine Farbe bereitgestellt werden soll, wobei die erste Maske ausgebildet wird, um den anderen Bereich als den vordefinierten Bereich zu bedecken; und
Aufbringen einer Materialflüssigkeit der einen definierten Bereich beschichtenden Maske auf das Aluminiummaterial mit der ersten Maske und Entfernen der ersten Maske, um die einen definierten Bereich beschichtende Maske im vordefinierten Bereich auszubilden.

9. Verfahren zur Herstellung eines gefärbten Aluminiumgegenstandes nach einem der Ansprüche 4 bis 8, wobei der Maskenausbildungsschritt umfasst:
einen Randausbildungsschritt zum Ausbilden eines Randes der einen definierten Bereich beschichtenden Maske mit einer ersten Maskenausbildungsflüssigkeit, für die eine UV-härtbare Tinte verwendet wird; und
einen Innenbereichsausbildungsschritt zum Ausbilden eines Maskeninnenbereichs, der vom Rand der einen definierten Bereich beschichtenden Maske umgeben ist, unter Verwendung einer zweiten Maskenausbildungsflüssigkeit, für die eine Tinte verwendet wird, die die Verdampfung von Lösungsmittel erfordert, um sich am Aluminiummaterial zu fixieren,
wobei im Randausbildungsschritt ein erster Flüssigkeitsausstoßkopf zum Ausstoßen der ersten Maskenausbildungsflüssigkeit verwendet wird, um die erste Maskenausbildungsflüssigkeit auf einen Bereich auszustoßen, der zum Rand der einen definierten Bereich beschichtenden Maske wird, und die erste Maskenausbildungsflüssigkeit, die auf das Aluminiummaterial aufgetroffen ist, mit Ultraviolettlicht bestrahlt wird, um den Rand der einen definierten Bereich beschichtenden Maske auszubilden, und
wobei im Innenbereichsausbildungsschritt ein zweiter Flüssigkeitsausstoßkopf zum Ausstoßen der zweiten Maskenausbildungsflüssigkeit verwendet wird, um die zweite Maskenausbildungsflüssigkeit auf den Bereich auszustoßen, der von dem Rand umgeben ist, der im Randausbildungsschritt ausgebildet wird, und den Maskeninnenbereich der einen definierten Bereich beschichtenden Maske auszubilden.

## Revendications

1. Procédé de production d'un article en aluminium coloré par coloration d'un matériau à base d'aluminium en utilisant au moins une tête d'éjection de liquide, le procédé comprenant les étapes de :
préparation d'un matériau à base d'aluminium sur lequel un revêtement anodisé est formé sur au moins une zone sur laquelle une couleur doit être appliquée ;
formation d'un masque de coloration qui recouvre une zone du matériau à base d'aluminium, une zone sur laquelle une couleur ne doit pas être appliquée en utilisant une encre durcissable sous UV ;
coloration du matériau à base d'aluminium sur la zone non recouverte par le masque de coloration avec une solution colorante qui utilise un solvant pouvant dissoudre le colorant ou qui utilise de l'eau en tant que solvant ;
séparation du masque de coloration par rapport au matériau à base d'aluminium après l'étape de coloration, et
conditionnement de la surface du matériau à base d'aluminium coloré.

2. Procédé de production d'un article en aluminium coloré selon la revendication 1, dans lequel le revêtement anodisé contient de fines pores et l'étape de conditionnement comprend le scellement des fines pores du revêtement anodisé.

3. Procédé de production d'un article en aluminium coloré selon la revendication 1 ou 2, dans lequel le revêtement anodisé contient de fines pores et l'étape de conditionnement comprend le scellement des fines pores du revêtement anodisé par chauffage.

4. Procédé de production d'un article en aluminium coloré selon l'une quelconque des revendications 1 à 3, dans lequel l'étape de formation de masque comprend la formation d'un masque de revêtement de zone définie qui recouvre une zone prédéfinie du matériau à base d'aluminium.

5. Procédé de production d'un article en aluminium coloré selon la revendication 4, dans lequel, dans l'étape de formation de masque, une encre acrylique durcissable sous UV est utilisée en tant que liquide de formation de masque et la tête d'éjection de liquide éjecte le liquide de formation de masque sur la zone prédéfinie afin de former le masque de revêtement de zone définie, et
dans lequel, dans l'étape de coloration, une solution colorante qui utilise un solvant pouvant dissoudre le colorant, ou qui utilise de l'eau en tant que solvant, est utilisée afin de colorer la zone non recouverte par le masque de revêtement de zone définie.

6. Procédé de production d'un article en aluminium coloré selon la revendication 4 ou 5, dans lequel, dans l'étape de formation de masque, une encre durcissable sous UV présentant la propriété de s'étirer après durcissement est utilisée en tant que liquide de formation de masque, et la tête d'éjection de liquide éjecte le liquide de formation de masque sur la zone prédéfinie afin de former le masque de revêtement de zone définie.

7. Procédé de production d'un article en aluminium coloré selon l'une quelconque des revendications 4 à 6, dans lequel, dans l'étape de formation de masque, une encre acrylique durcissable sous UV est utilisée afin de former le masque de revêtement de zone définie sur le matériau à base d'aluminium gravé avec une solution acide.

8. Procédé de production d'un article en aluminium coloré selon l'une quelconque des revendications 4 à 7, dans lequel l'étape de formation de masque comporte :
la formation d'un premier masque avec le liquide de formation de masque éjecté sur une zone autre que la zone prédéfinie dans la zone de coloration cible du matériau à base d'aluminium sur laquelle une couleur doit être appliquée, le premier masque étant formé afin de recouvrir la zone autre que la zone prédéfinie ; et
l'application d'un matériau liquide du masque de revêtement de zone définie sur le matériau à base d'aluminium comportant le premier masque, et l'élimination du premier masque afin de former le masque de revêtement de zone définie sur la zone prédéfinie.

9. Procédé de production d'un article en aluminium coloré selon l'une quelconque des revendications 4 à 8, dans lequel l'étape de formation de masque comporte :
une étape de formation de rebord destinée à former un rebord du masque de revêtement de zone définie avec un premier liquide de formation de masque pour lequel une encre durcissable sous UV est utilisée ; et
une étape de formation de zone interne destinée à former une zone interne de masque entourée par le rebord du masque de revêtement de zone définie, en utilisant un second liquide de formation de masque pour lequel il est utilisé une encre qui nécessite l'évaporation du solvant afin de se fixer elle-même sur le matériau à base d'aluminium,
dans lequel, dans l'étape de formation de rebord, une première tête d'éjection de liquide destinée à éjecter le premier liquide de formation de masque est utilisée afin d'éjecter le premier liquide de formation de masque sur une zone qui devient le rebord du masque de revêtement de zone définie, et le premier liquide de formation de masque reçu sur le matériau à base d'aluminium est soumis à de la lumière UV afin de former le rebord du masque de revêtement de zone définie, et
dans lequel, dans l'étape de formation de zone interne, une seconde tête d'éjection de liquide destinée à éjecter le second liquide de formation de masque est utilisée afin d'éjecter le second liquide de formation de masque sur la zone entourée par le rebord formé dans l'étape de formation de rebord, et de former la zone interne de masque du masque de revêtement de zone définie.
